

April 15, 1947.

R. E. HARR

2,418,932

METHOD OF MAKING ENAMEL COATED ARTICLES

Filed Nov. 13, 1940

FIG. 1



FIG. 2



INVENTOR  
R. E. HARR

BY *Emery Robinson*  
ATTORNEY

## UNITED STATES PATENT OFFICE

2,418,932

## METHOD OF MAKING ENAMEL COATED ARTICLES

Russel E. Harr, Chicago, Ill., assignor to Western Electric Company, Incorporated, New York, N. Y., a corporation of New York

Application November 13, 1940, Serial No. 365,453

4 Claims. (Cl. 204—38)

1

This invention relates to methods of making enamel coated articles.

An object of the invention is the provision of improved methods for the production of articles having a metal base and a smooth, highly ornamental and serviceable coating of vitreous enamel on the base.

The present invention is particularly adapted to the production of articles such as the number plates incorporated in telephone dials, which comprise a base and a coating of vitreous enamel on the portions of the base that are exposed in the dial assembly. It is desirable to make the base from a material which is durable, inexpensive, and readily formable into required shape. Iron and certain grades of steel meet these requirements adequately but it is impractical to produce directly on these ferrous materials an enamel coating having all of the properties desired in articles of this type. The enamel on number plates must be highly adherent to withstand rough usage in service and it is particularly important that the enamel have a smooth, even and unbroken surface. Number plates are often exposed to dirt-laden atmospheres in service and under these conditions even minute imperfections in the enamel surface tend to accumulate dust, dirt, lint and the like, which mars the appearance of the plates and also detracts from their utility.

Because of these requirements and limitations, it has been customary to employ intermediate layers, or undercoatings, of different metals between the ferrous base and the enamel. In one of these constructions, a coating of copper is applied on the ferrous base, a layer of nickel-iron alloy is applied on the copper, and the vitreous enamel coating is then applied on the alloy layer. The present invention relates to an improved process for forming this nickel-iron alloy.

In accordance with one embodiment of the invention, a base of desired shape is first formed of sheet iron and then copper plated, after which a layer of nickel-iron alloy is electrodeposited on the copper. The alloy layer is produced in an electrolytic solution comprising nickel-sulfate, ferrous sulfate, nickel and iron anodes immersed in the solution, and a porous container immersed in the solution and containing small particles of metallic iron. The vitreous enamel is applied on the alloy layer and the base is then fired at a suitable temperature to fuse the enamel into a coating.

A more complete understanding of the invention may be had by reference to the following de-

2

tailed description, taken in conjunction with the accompanying drawing, in which

Fig. 1 is a plan view of a number plate embodying the invention, and

Fig. 2 is an enlarged sectional view of the number plate taken on the line 2—2 of Fig. 1.

In the first operation for producing a complete number plate in accordance with this invention, a ring or base 10 is formed from ferrous sheet metal. Various grades of steel or iron are suitable for this purpose and the material is selected primarily on the basis of durability, cost and formability.

After the ring-shaped base is formed, it is cleaned by the usual methods, such as immersion in alkaline and acid solutions, and then completely coated with a layer of copper 11. The copper can be applied conveniently in a conventional copper cyanide electroplating process and a coating weight around 20 milligrams per square inch is generally satisfactory.

In the next operation, a nickel-iron alloy 12 is electrodeposited over the copper in a uniform layer. The iron content of the alloy should be between .50% and 10.0% with the balance nickel and the best results are secured with an alloy having an iron content around 1.5%.

To apply an alloy containing 1.5% iron and the balance nickel, an aqueous bath of the following composition is first prepared:

|                  | Ounces per gal.<br>of solution |
|------------------|--------------------------------|
| Nickel sulphate  | 24.0                           |
| Sodium chloride  | 3.0                            |
| Boric acid       | 4.0                            |
| Ferrous sulphate | .0666                          |

The solution is placed in the tank of a conventional electroplating apparatus. This tank is lined with rubber or similar material and soluble anodes of pure nickel and of pure iron are suspended in the solution from the electrode bars with the iron and nickel anodes arranged in parallel.

A quantity of metallic iron, preferably in the form of small particles, is also immersed in the solution but not connected electrically to the anode or cathode bars. Small metallic iron shot or grit, around 90 mesh in size, is particularly suitable for this purpose and good results are obtained by enclosing the iron particles in a porous container of non-conducting material, such as a cloth bag, and then suspending the container in the solution. Several bags of iron particles may be suspended in the solution, the distribution 55 of the bags depending upon the size and arrange-

## 3

ment of the tank. The presence of oxidized iron (ferric oxide) in the plating solution produces an alloy which causes enameling defects when enamel is later applied thereto. The addition of metallic iron to the bath reduces the ferric oxide to ferrous oxide which is not detrimental to the production of a satisfactory nickel-iron alloy.

The copper plated bases are then suspended in the solution and current applied until an alloy coating of desired weight is electrodeposited on the copper. The process is operated at a temperature between 135° F. and 145° F. and a current density between 40 and 60 amperes per square foot of cathode surface. The means of these values are used preferably.

The above temperature and current density ranges are critical and their interrelation is important. A variation in current density, for example, will affect the proportions of iron in the deposited alloy for a given solution and temperature, as well as the properties of the alloy, and for best results the above combination of solution concentrations, operating temperatures and current densities should be maintained. The described solution will produce an alloy containing about 1.5% iron. If an alloy having a lower or higher iron content is desired, the bath is correspondingly adjusted by the use of less or more ferrous sulfate or anodes.

After the copper and the alloy coatings have been deposited on the base, the base is ready to receive the enamel, which is applied only on the face of the ring, or the portion exposed in service, in order to minimize the cost of the article and also to facilitate the maintenance of over-all dimensional tolerances.

A coating of white enamel 13, such as a lead boro-silicate enamel opacified with arsenic oxide, is applied first. The enamel is distributed on the alloy surface either in the form of dry powder or by a wet process in which the enamel particles are mixed with water and a flotation agent, such as clay. The base is then fired at a temperature around 1600° F. for about three and one-half minutes to fuse the enamel.

Identifying characters in contrasting colors are usually required to complete the plate. The application of these characters usually involves repeated refiring of the initial enamel coating and this practice tends to aggravate any roughness or other imperfections present in the initial coating.

One type of plate, shown in the drawing, has a background 14, letters 15 and numerals 16. These characters are produced with an inky suspension of colored metallic oxides or frits in a vehicle such as linseed oil and are applied on the surface of the white enamel by a printing operation. The background, which may be blue or black, is applied first and the plate is then baked at about 1300° F. to harden the ink so that it will not be marred in subsequent printing operations. The letters, which are usually black, are then applied and the plate is then again baked at a temperature of about 1300° F. The numerals are usually colored red and are applied in the same manner, after which the entire plate is again fired to fully mature the ceramic ink which requires exposure to a temperature around 1300° F. for approximately 4.5 minutes.

The resultant enamel coating is highly adherent and has a smooth and continuous surface. In enameling number plates the peripheral edge portions of the enamel surface are critical and plates produced by prior methods have tended

to develop a defect commonly known as "edge pimpling" in these areas. These pimples may be very small and difficult to detect, but after a period of service, they accumulate dirt and other foreign material to form smudges which are very difficult to remove, particularly because the number plates are not readily accessible for cleaning after they are assembled in a dial.

The nickel-iron alloy layer produced as herein described causes the enamel to fuse into a smooth coating without the formation of pimples anywhere on the coating surface. The initial coat, of white enamel, is glassy and free of pimples and these desirable surface conditions are preserved during any refiring operations employed in the application of characters on the enamel. The action of the metallic iron on deposition of the alloy under the prescribed operating conditions contributes largely to the desired alloy properties and, as stated, this metallic iron is preferably provided in the form of small particles.

For most applications, a coating weight of 20 milligrams per square inch for both the copper and the alloy is satisfactory, although it may be desirable to vary these values somewhat for different enamel compositions, and, in general, the copper and alloy layers should be of about equal weight.

Although the invention has been described in connection with the manufacture of number plates for telephone dials, it will be apparent that it is equally applicable to other ornamented enameled articles and it is to be understood that the invention is limited only by the scope of the appended claims.

## What is claimed is:

1. A method of coating an article with a vitrifiable material which comprises electrodepositing a layer of nickel-iron alloy containing from .5% to 10% of iron on the article in a nickel sulfate, ferrous sulfate solution, employing a nickel anode and an iron anode, maintaining a quantity of metallic iron in a subdivided state in the solution, applying a vitrifiable material on the alloy layer, and heating the article to fuse the vitrifiable material to form a smooth coating.

2. A method of coating an article with a vitrifiable material which comprises electrodepositing a layer of nickel-iron alloy containing from .5% to 10% of iron on the article in a nickel sulfate, ferrous sulfate solution, employing a nickel anode and an iron anode, placing a quantity of metallic iron in addition to the iron anode in the solution, applying a vitrifiable material on the alloy layer, and heating the article to fuse the vitrifiable material to form a smooth coating.

3. A method of coating an article with a vitrifiable material which comprises applying a layer of copper on the article, electrodepositing a layer of nickel-iron alloy containing from .5% to 10% of iron on the article in a nickel sulfate, ferrous sulfate solution, employing a nickel anode and an iron anode, placing particles of metallic iron in the solution during the electrodeposition, applying a current density of between 40 and 60 amperes per square foot to the surface being coated at a temperature of 135° F. to 145° F., covering the surface of the electrodeposited alloy with a vitrifiable material, and heating the article to fuse the vitrifiable material to form a smooth coating.

4. A method of coating a ferrous base article with a vitrifiable material which comprises applying a layer of copper to the ferrous base,

electrodepositing a layer of nickel-iron alloy containing from .5% to 10% of iron on the copper layer and a nickel sulfate, ferrous sulfate solution, employing a nickel anode and an iron anode, placing a quantity of metallic iron in a subdivided state in the solution, applying a vitrifiable material on the alloy layer, and heating the article to fuse the vitrifiable material to form a smooth coating.

RUSSEL E. HARR.

## REFERENCES CITED

The following references are of record in the file of this patent:

## UNITED STATES PATENTS

| Number    | Name         | Date           |
|-----------|--------------|----------------|
| 708,363   | Ketcham      | Sept. 2, 1902  |
| 1,522,291 | Eimen        | Jan. 6, 1925   |
| 1,837,355 | Burns et al. | Dec. 22, 1931  |
| 2,020,476 | Scott        | Nov. 12, 1935  |
| 1,885,700 | Fink         | Nov. 1, 1932   |
| 1,127,966 | Cowper-Coles | Feb. 9, 1915   |
| 2,131,427 | Crowder      | Sept. 27, 1938 |
| 1,007,388 | Ramage       | Oct. 31, 1911  |

## OTHER REFERENCES

Cir. Bureau of Standards, No. 100 (1924), p. 9,  
15 204-49.